

Oct. 10, 1967

E. A. MIZIKAR ET AL  
METHOD OF PRODUCING STEEL STRIP OF UNIFORM  
THICKNESS BY DIRECT COATING

3,345,738

Filed Nov. 10, 1964

2 Sheets-Sheet 1



Fig. 1a.

Fig. 1b.



FIG. 2a



FIG. 2b



FIG. 2c



FIG. 2d



FIG. 2e



FIG. 2f



FIG. 2g

INVENTORS.  
EUGENE A. MIZIKAR  
WITOLD M. WOJCIK &  
KUN LI

BY

*JR Harris*  
their ATTORNEY

Oct. 10, 1967

E. A. MIZIKAR ET AL  
METHOD OF PRODUCING STEEL STRIP OF UNIFORM  
THICKNESS BY DIRECT COATING

3,345,738

Filed Nov. 10, 1964

2 Sheets-Sheet 2



FIG. 3a



FIG. 3b



FIG. 3c



FIG. 3d



FIG. 3e



FIG. 3f



FIG. 3g



FIG. 4

INVENTORS.  
EUGENE A. MIZIKAR  
WITOLD M. WOJCIK &  
KUN LI

BY

*JR Davis*

their ATTORNEY

1

3,345,738

**METHOD OF PRODUCING STEEL STRIP OF UNIFORM THICKNESS BY DIRECT CASTING**  
Eugene A. Mizikar, Witold M. Wojcik, and Kun Li,  
Pittsburgh, Pa., assignors to Jones & Laughlin Steel  
Corporation, Pittsburgh, Pa., a corporation of Penn-  
sylvania

Filed Nov. 10, 1964, Ser. No. 410,066  
9 Claims. (Cl. 29—528)

## ABSTRACT OF THE DISCLOSURE

This invention is directed to a method of producing steel strip of uniform thickness by direct casting so that the strip can withstand rolling to the desired gauge. A uniform thickness is achieved by impressing on the skin of the strip as it is formed a pattern of indentations defining a regular network finer in mesh than the random hill and hollow network which the skin solidifies into in the absence of such impressed indentations. The strip as a result of being uniformly thick will be able to withstand rolling without breaking.

This invention relates to the casting of metal strip. It is more particularly concerned with the casting of low carbon steel strip suitable for subsequent rolling and is described hereinafter with particular reference to that material.

Steel strip is conventionally made by casting molten steel of the desired composition into ingots and then reducing the ingots by successive hot rollings. A large tonnage of steel strip is cold rolled to final gauge, but the starting material for this cold rolling is hot band, so called, which is strip hot rolled to an intermediate gauge. Attempts have been made to eliminate the casting of the steel into ingots by continuously casting the steel through a mold. Attempts have also been made to eliminate both the casting of the steel into ingots and some of the rolling by casting the steel directly into a pair of rolls or moving belts, to produce a cast product requiring little further reduction. While these attempts have had some degree of success with bar shapes, they have not resulted in a commercial process for the production of strip of any considerable width. A seemingly attractive process for the direct production of wide thin strip is that of solidifying the steel against a chill, that is, a surface much colder than the molten steel, and stripping or removing it therefrom. Such processes are exemplified in Wagner Patent 1,025,848 and Sendzimir Patent 2,074,812, both of which produce strip by rotating the chill surface in a pool of molten metal. A difficulty with previously known processes of this type is that if steel strip is cast thin enough to be easily removed from the chill, it is not at all uniform in thickness and breaks up in subsequent rolling.

It is an object of our invention to provide a process of casting thin steel strip sufficiently uniform in thickness to withstand rolling to the desired gauge. It is another object to provide a process of casting steel strip of minimum surface irregularity. It is another object of our invention to provide a process of casting steel strip having a controlled surface pattern. Other objects of our invention will appear in the following description of an embodiment thereof presently preferred by us.

Stated briefly, our process comprises bringing a chill surface into contact with molten steel so that a thin skin of steel solidifies thereon and creating in that skin a surface pattern of distributed point indentations. The solidified steel is then stripped from the chill surface and sub-

2

sequently hot rolled to the desired gauge. To produce cast strip continuously, it is necessary to move the chill with respect to the molten steel and we provide this movement in conventional ways, such as by forming the chill into a cylinder rotating about its axis with a portion of its surface dipping into the molten steel. Conventionally the chill is made of copper, and is fluid cooled.

Certain aspects of our invention will be more easily understood by reference to the attached figures. FIGURE 1-a is the outer surface, not in contact with the chill, of low carbon steel solidified against a smooth chill in the manner known to the prior art. FIGURE 1-b is the surface of the steel of FIGURE 1-a in contact with the chill. FIGURES 2-a through 2-g are chill surface patterns with which we have experimented and which we describe hereinafter. FIGURES 3-a through 3-g are the surfaces of cast low carbon steel strip in contact with the chills having the surface patterns of FIGURES 2-a through 2-g respectively. FIGURE 4 is the outer surface of the steel of FIGURE 3-c.

When a metal, such as low carbon steel, is solidified in a thin layer against a smooth chill surface, neither the surface of the steel adjacent the chill nor the opposite surface of the strip is smooth. By low carbon steel we mean steel having a carbon content not above about 0.12%, and otherwise of the composition conventional for hot or cold rolled sheet and strip, such as A.I.S.I. grade 1008. The outer surface of such steel is illustrated in FIGURE 1-a. The surface is one of hills 1-1 separated by interconnecting hollows 2-2. The surface of the same steel in contact with the chill is illustrated in FIGURE 1-b. It also displays hills 3-3 and hollows 4-4, which correspond generally to the hills and hollows of FIGURE 1-a. The surface area within a mesh formed by interconnecting hollows 4-4 may be of the order of a square inch. The difference in strip thickness between hills and hollows is substantial. When this strip is rolled it breaks up along the lines of the hollows because of the unequal stresses which the rolling induces.

It is our view that this undesirable pattern or network of hills and hollows results from the way the steel solidifies against the chill. Initially a thin layer of steel solidifies against the chill and is quickly cooled to a low temperature while successive layers of steel solidify on top of it. As these superimposed layers cool, they shrink, setting up a system of stresses in the cast strip parallel to the chill face. The shrinkage stresses in the metal relatively remote from the chill face tend to bend the cast material away from the chill face wherever conditions permit such bending. One condition permitting such bending is, of course, fracture of the skin. Presumably, such fractures are initiated in inhomogeneities, such as non-metallic inclusions in the steel.

Whatever their cause, random fractures of the skin are followed by uplifting of the edges formed by the fractures and frequent partial refilling of the breaks with liquid metal. The consequences of this separation is a substantial decrease in the rate of heat transfer from the metal to the chill surface along the fractures, resulting in slower growth of skin there than in those areas remaining in direct contact with the chill surface. This is believed to be the mechanism which leads to the hill and hollow pattern on strip cast against a smooth chill surface.

We have found that this hill and hollow network is suppressed if a pattern of distributed point indentations is deliberately imposed on the solidifying skin. These point indentations may be connected by line indentations if desired, but a pattern of line indentations which do not define a network is not effective. The point indentations must be spaced so that the network or grid they define is of finer mesh than the network of hills and hollows which

it is desired to suppress. Indenting of the solidifying surface of the cast steel is most conveniently accomplished by knurling the surface of the chill. It is conceivable that the steel solidifies in a thin skin surrounding the points of the knurled surface and subsequently fractures at or around those points, or that the skin does not actually fracture, but merely yields between those points so as to relieve the shrinkage stresses. It is also conceivable that the indentations increase the uniformity of heat transfer over the contact area between the chill and the solidifying strip. If the chill surface is indented in a pattern defining a network smaller in mesh than that of the random hill and hollow network, the contact between metal and chill is now provided by the numerous uniformly distributed small chill areas. These small areas form active sites for solidification with each small area behaving as a smooth chill. Since the areas of contact are uniformly and finely distributed, the hills and hollows on the outer surface of strip cast on such a chill surface will be so numerous and close to one another that the strip will appear to be of uniform thickness. While the theories above set out are believed by us to be correct, we do not consider ourselves bound thereby.

FIGURES 2-a through 2-g hereof represent seven configurations of chill surface we have employed. The surface of FIGURE 2-a is provided with parallel V-grooves 5-5 which do not define a network. This chill surface, like a smooth chill surface, is not effective for our process. The remaining six FIGURES 2-b through 2-g are of knurled surfaces of various types and spacings. FIGURES 2-b, 2-c and 2-d may be described as fine, medium and coarse knurled surfaces respectively, and comprise diamond knurls formed by cutting a family of parallel V-grooves 6-6 and crossing them with another family of parallel V-grooves 7-7 so as to form a surface of points 8-8. The reference characters have been applied only to FIGURE 2-d, but it will be understood that the knurls of FIGURES 2-b and 2-c are formed in the same way. Surface 2-e comprises shallow pyramids 9-9 and is formed in the same way as the knurled surfaces, but with wider angle intersecting V-grooves 10-10 and 11-11 respectively. The surfaces of FIGURES 2-b through 2-e form a series in which the spacing between points and the depth of the grooves increase from the relatively small values of FIGURE 2-b to the relatively large values of FIGURE 2-e. The square waffle surface of FIGURE 2-f is formed by cutting intersecting families of V-grooves 12-12 and 13-13 of diminished groove angles so that the chill surface consists of separate squares 14-14 covering the major portion of the chill area. The diamond waffle surface of FIGURE 2-g is similar, but is formed with intersecting grooves 15-15 and 16-16 of wider V-angle so that the surface squares 17-17 occupy only a minor portion of the chill area. Table I lists the groove depth, angle of groove, and grid density of the surface illustrated in FIGURES 2-a through 2-g.

TABLE I

| Surface         | Groove Depth, Inch | Angle of Groove, Degrees | Grid Density                      |
|-----------------|--------------------|--------------------------|-----------------------------------|
| Figure 2-a----- | 0.040              | 60                       | 4 grooves/inch.                   |
| Figure 2-b----- | 0.008              | 84                       | 1,600 points/(inch). <sup>2</sup> |
| Figure 2-c----- | 0.017              | 80                       | 576 points/(inch). <sup>2</sup>   |
| Figure 2-d----- | 0.025              | 72                       | 256 points/(inch). <sup>2</sup>   |
| Figure 2-e----- | 0.020              | 160                      | 25 pyramids/(inch). <sup>2</sup>  |
| Figure 2-f----- | 0.030              | 60                       | 25 blocks/(inch). <sup>2</sup>    |
| Figure 2-g----- | 0.040              | 120                      | 16 diamonds/(inch). <sup>2</sup>  |

FIGURES 3-a through 3-g represent steel strip surfaces which were cast in contact with chills having surface textures of FIGURES 2-a through 2-g respectively. The surface of FIGURE 3-a is not greatly different from that of FIGURE 1-b except for the superimposed pattern of ridges 18-18 corresponding to the grooves 5-5 of FIGURE 2-a. It displays hills 19-19 and hollows 20-20

relatively extensive in area. The strip of 3-b also shows hills 21-21, although of lesser height, against a relatively level area 22. The strip of FIGURE 3-c, cast on the medium knurled surface of FIGURE 2-c, displays only a few faint traces 23-23 of a network pattern while that pattern is effectively suppressed in the surfaces of FIGURES 3-d through 3-g.

It is undesirable to indent the surfaces of the cast strip any more than is necessary because deeper indentations require more rolling of the cast strip to obliterate. We prefer, therefore, to impress on the skin of the cast strip the medium knurl pattern of FIGURE 2-c, or its equivalent. From Table I it may be seen that the groove depth of this pattern on the chill surface is .017 inch and that 15 the grid density is 576 points per square inch.

The effectiveness of the medium knurled chill surface of FIGURE 2-c in improving the outer surface of the strip is shown in FIGURE 4 which illustrates the outer surface of the steel of FIGURE 3-c. It displays only 20 relatively shallow hills and hollows 25-25 and 26-26 respectively. This surface contrasts very favorably with that of FIGURE 1-a which is the outer surface of steel cast on a smooth chill. The ratio of thickest to thinnest section of the steel of FIGURE 1 is about 4 to 1, far 25 greater than the thickness ratio of 2 to 1 for the steel of FIGURE 4. The steel of FIGURE 1 could not be rolled without tearing, whereas, that of FIGURE 4 was rolled without difficulty.

Low carbon steel strip cast against a medium knurled 30 chill of FIGURE 2-c to a thickness of about 0.3 inch was grit blasted to remove scale, heated to a temperature of 2200° F., soaked at that temperature for 15 minutes, and then given two passes each of about 50% reduction through smooth rolls. The resulting strip of about .090 35 inch thickness and at a temperature of about 1600° F. was water spray quenched to about 1000° F. and allowed to cool in air to room temperature. The strip was grit blasted and pickled lightly to remove rolling scale and was then cold reduced to about .035 inch. This material 40 in the fully annealed condition exhibited yield strengths of 31,000 to 33,000 p.s.i., ultimate strengths of 46,000 to 48,000 p.s.i., and uniform elongations of about 35%.

It is desirable to cast the steel at a temperature no higher than is necessary to maintain it in a molten state. 45 We prefer to cast ordinary low carbon steel at a temperature of about 2800° F. and no higher than 2950° F. Higher temperatures cause steeper temperature gradients in the cast strip and result in less even thickness. Alloy steels should be cast close to their liquidus temperatures.

50 The most uniform thickness of low carbon steels is obtained when the carbon content of the steel is below about 0.06%. However, up to about 0.14% carbon the surface irregularities are not objectionable.

We claim:

55 1. In the process of producing directly cast metal strip by bringing molten metal into contact with a chill so as to cause rapid solidification of a skin of metal against the chill surface, thereafter withdrawing the solidified steel from the chill and subsequently rolling the steel to 60 reduce its thickness, the improvement comprising impressing on that skin as it is formed a pattern of indentations defining a regular network finer in mesh than a random hill and hollow network which the skin would solidify into in the absence of the impressed indentations.

65 2. The process of claim 1 in which the meshes of the defined network are substantially equal in size.

3. The process of claim 1 in which the indentations are point indentations.

4. The process of claim 1 in which the indentations 70 are point indentations uniformly spaced from each other.

5. The process of claim 1 in which the indentations are point indentations and number not more than about 576 per square inch.

6. The process of claim 1 in which the depth of the 75 pattern is at least about .017 inch.

7. The process of claim 1 in which the indentations are point indentations and at least some of them are connected together to form line indentations.

8. The process of claim 1 in which the strip is reduced by hot rolling in an amount sufficient to obliterate the impressed indentation pattern.

9. The process of claim 1 in which the strip after it is withdrawn from the chill surface is first reheated to rolling temperature and then reduced by hot rolling in an amount sufficient to obliterate the impressed indentation pattern.

## References Cited

## UNITED STATES PATENTS

|           |         |                |          |
|-----------|---------|----------------|----------|
| 2,577,423 | 12/1951 | Ludwig et al.  |          |
| 3,101,533 | 8/1963  | Rosbach        | 29—528 X |
| 3,145,119 | 8/1964  | Laforce et al. | 29—528 X |
| 3,147,521 | 9/1964  | Boehm          | 29—528 X |

JOHN F. CAMPBELL, Primary Examiner.

10 P. M. COHEN, Assistant Examiner,